

March 18, 1930.

W. HOSKINS, JR

1,750,754

HECTOGRAPH BLANKET

Filed July 2, 1928

Fig. 1



Fig. 2.



Inventor:

William Hoskins Jr.

By Wilkinson, Husley, Bryan & Knight  
Atty's

## UNITED STATES PATENT OFFICE

WILLIAM HOSKINS, JR., OF CHICAGO, ILLINOIS, ASSIGNOR TO DITTO INCORPORATED,  
OF CHICAGO, ILLINOIS, A CORPORATION OF ILLINOIS

## HECTOGRAPH BLANKET

Application filed July 2, 1928. Serial No. 290,037.

This invention relates to hectograph sheets or blankets or similar means which embody the same characteristic principles of operation.

5 The principal object of the present invention is to provide a hectograph sheet or blanket having the customary coating of suitable material for the absorption of ink, which will produce a large number of good copies, 10 will not harden or dry out and which is substantially opaque whereby the ink absorbed inwardly from the surface renders it visibly clean.

The use of hectograph sheets or blankets 15 is well known for reproducing copies of typed, written or other like matter, and is known to involve the use of a coating usually of a mixture of glue and glycerin applied on a backing sheet. The written matter to be 20 reproduced is produced originally in a special kind of ink adapted for this use which is absorbed by and maintained on the surface of the glue and glycerin coating when the sheet is pressed in contact therewith. Relatively 25 large numbers of copies may be made by placing additional sheets in contact with the blanket which gives up the ink to produce reproductions of the original thereon.

After periods of standing the glue-glycerin 30 coating possesses a characteristic of absorbing the ink inwardly from the surface whereby the surface is rendered clean and fresh and capable of reuse for producing additional and different copies.

35 In order to produce good copies it is found desirable, after the original has been offset on to the glue-glycerin blanket, to ascertain by inspection the quality of the offset, that is to make sure that the copy has been accurately transferred and is in proper condition to take additional copies from. It is also found, however, that the ink which has been absorbed inwardly of the surface as occasioned by former use of the blanket becomes diffused 45 throughout the volume of the coating material, and due to the transparent nature of the glue-glycerin coating, is readily visible presenting a background similar in color to that of the ink employed. The presence of the ink 50 colored background renders it very difficult

to readily detect the outline of the offset matter on to the surface of the blanket. This difficulty is encountered after the blanket has been used a relatively few number of times because the absorbed ink quickly forms the 55 background against which no substantial contrast can be made.

It has been found desirable, therefore, to incorporate in the blanket coating material, a pigment which will have sufficient hiding 60 power to render the blanket substantially opaque and of such contrasting color that the freshly inked surface will be readily detectable upon inspection. This involves considerable difficulty, however, on account of the 65 fact that many pigments or inert powdered substances which might be employed for this purpose tend to dilute the ink absorbing medium with a consequent diminishing of the effect and functioning of the blanket, and further tend to render the coating short or 70 crumbly in character and to cause premature drying or hardening thereof.

It has been only through long experimenting that a substance having the desirable 75 properties has been found, that is, having such high hiding power that it will produce a coating substantially opaque when employed in quantities proportionally so small that its presence has substantially no effect on the 80 properties of the blanket.

The present invention accordingly involves the use of titanium oxide which is a white inert powdered substance having an extremely high hiding power. Titanium oxide is 85 found in practice to produce white blankets highly efficient in service when the titanium oxide is added in proportions of approximately 1/2 of 1% of the contents of the glue-glycerin composition. This small amount of titanium oxide is found to produce a very white blanket, more opaque for the quantity used than any other substance found and when employed in the proportions specified 90 will produce a blanket which, after a period 95 of standing and absorption of the ink, presents a clean white surface capable of ready inspection of the offset imprint thereon.

The present invention contemplates the introduction of the titanium oxide by any de- 100

sired method, it being found well in practice to mix it in with the glue-glycerin composition by the use of mixing rolls, it being found that the pulverizing and mixing action of the rolls produces superior results. The small amount necessary to produce the desirable opaque character of the coating is found to have substantially no effect on the properties of the blanket material and consequently results in a blanket having all of the usual desirable properties of hectograph blankets plus that of ready visibility of the fresh imprint on its surface.

In order to better understand this invention, reference is here made to the accompanying drawing which discloses a hectograph roll constructed in accordance with the present invention in which—

Figure 1 is an enlarged cross sectional view with the materials employed indicated on the drawing, and

Figure 2 is a perspective view of a roll.

As shown in the drawing, the coating of the described kind is applied to the flexible backing sheet in a manner disclosed.

It is to be understood that the above disclosure is merely given by way of example as one form of the invention and is not to be considered as limiting the invention in any respect.

The true scope of the invention will be ascertained from an understanding of the operation of advantages of the present disclosure with the knowledge that it is one embodiment thereof. The scope of the invention is particularly pointed out in the appended claims.

I claim:

1. A hectograph blanket, comprising, a backing sheet and a coating on one face thereof of the usual glue and glycerine composition, said coating containing titanium oxide.

2. A hectograph blanket comprising, a backing sheet and a coating on one face thereof of the usual glue and glycerine composition, said coating containing substantially  $\frac{1}{2}$  of 1% of titanium oxide.

Signed at Chicago, Illinois, this 23rd day of June, 1928.

WILLIAM HOSKINS, JR.